

## UNITED STATES PATENT OFFICE

2,268,427

## ABRASION RESISTING ALLOY

Robert W. Schlumpf, Houston, Tex., assignor to  
 Hughes Tool Company, Houston, Tex., a corporation of Delaware

No Drawing. Application November 10, 1941,  
 Serial No. 418,595

## 2 Claims. (Cl. 75—126)

My invention relates to a combination of metals to be employed in the construction of a wear resisting alloy.

The invention is designed for use in the casting of tools and other objects which are subject to extreme wear and abrasion in use. The principal object of the invention is to provide a ferrous alloy which is particularly hard and abrasion resisting.

In making up my hard metal composition I have developed a formula employing ingredients fused together in approximately the following proportions:

|            | Per cent               |
|------------|------------------------|
| Carbon     | 1.50-4.00              |
| Manganese  | 1.00-3.00              |
| Silicon    | 0.50-2.50              |
| Chromium   | 3.00-7.00              |
| Molybdenum | 5.00-10.00             |
| Vanadium   | 1.00-3.00              |
| Boron      | 0.50-1.50              |
| Iron       | Balance to make up 100 |

These ingredients alloyed together within the ranges indicated above will produce a material extremely hard but somewhat brittle. The alloy may be cast but it is not malleable. The ingredients may be mixed approximately within the ranges set out in the above example, and although variance within these limits is not material I have found that the following proportion of the ingredients is particularly satisfactory in the production of wear resisting tools or devices:

|            | Per cent               |
|------------|------------------------|
| Carbon     | 3.62                   |
| Manganese  | 2.20                   |
| Silicon    | 2.20                   |
| Chromium   | 4.50                   |
| Molybdenum | 8.20                   |
| Vanadium   | 2.40                   |
| Boron      | 1.00                   |
| Iron       | Balance to make up 100 |

In the construction of this alloy the various materials in the proportions approximately as indicated are fused together and cast into the form in which they are to be used. The alloy is particularly designed for use in nozzles which are subjected to the action of sand or other similar hard material brought into contact therewith. Sand blast nozzles, in which the sand is forcibly brought into impact with the material of the nozzle, may be made of this material, and it has been found that the alloy will resist wear for a materially longer period of time than other alloys now in common use.

What is claimed as new is:

1. A hard abrasion resisting ferrous metal alloy comprising the following ingredients fused together in approximately the proportions stated below:

|            | Per cent               |
|------------|------------------------|
| Carbon     | 1.50-4.00              |
| Manganese  | 1.00-3.00              |
| Silicon    | 0.50-2.50              |
| Chromium   | 3.00-7.00              |
| Molybdenum | 5.00-10.00             |
| Vanadium   | 1.00-3.00              |
| Boron      | 0.50-1.50              |
| Iron       | Balance to make up 100 |

2. A cast ferrous hard metal object made up of ingredients alloyed together in approximately the following proportions:

|            | Per cent               |
|------------|------------------------|
| Carbon     | 3.62                   |
| Manganese  | 2.20                   |
| Silicon    | 2.20                   |
| Chromium   | 4.50                   |
| Molybdenum | 8.20                   |
| Vanadium   | 2.40                   |
| Boron      | 1.00                   |
| Iron       | Balance to make up 100 |

ROBERT W. SCHLUMPF.